

Oct. 26, 1926.

1,604,576

F. C. MATHERS ET AL

PRODUCTION BY CARBONATION AND THE ADDITION OF SULPHATES OF PLASTIC  
MATERIALS HAVING AN INITIAL QUICK SET

Filed July 25, 1923



Inventors

Frank C. Mathers

Russel L. Hardy

By *Duan P. Tashy*

Attorney

## UNITED STATES PATENT OFFICE.

FRANK C. MATHERS, OF BLOOMINGTON, INDIANA, AND RUSSEL L. HARDY, OF WOODVILLE, OHIO, ASSIGNEES TO NATIONAL LIME ASSOCIATION, OF WASHINGTON, DISTRICT OF COLUMBIA, A CORPORATION OF THE DISTRICT OF COLUMBIA.

PRODUCTION BY CARBONATION AND THE ADDITION OF SULPHATES OF PLASTIC MATERIALS HAVING AN INITIAL QUICK SET.

Application filed July 25, 1923. Serial No. 653,718.

Our invention relates to the production of plastic materials which have quick initial setting properties and which are adapted to be used in the making of mortars, plasters, shaped articles such as blocks, boards and the like.

The use of calcined gypsum for plastering purposes is well known. Gypsum sets so quickly that it is necessary to add varying proportions of a retarding agent to delay the set sufficiently to allow the workmen time to get the plaster on the wall. In addition to this objection, gypsum has a number of other serious objections and disadvantages. For example, the material is difficult to work, owing to its lack of plasticity and, as compared to lime, its low sand-carrying capacity. It has been proposed to use lime for plastering purposes but this material has one serious disadvantage namely—it is necessary to wait a considerable period of time—twenty to twenty-four hours—for each coat to acquire what may be termed its initial set, by which it becomes sufficiently strong, firm and dry so that the succeeding coat may be applied. This is quite a serious objection since it requires the removal of scaffolds from one room to another between the application of the various coats, if the workmen are not to suspend work entirely.

The term "initial set" is used to indicate that condition of the lime plaster which makes it suitable for the application of the second or brown coat. It is not necessarily hard in this condition, but is firm, strong and rigid enough to support the weight of the second coat and withstand the pressure necessary in the application of the second coat. This is distinguished from the term "hardening" in that the latter refers to the condition of the mortar after it has undergone practically all the physical and chemical changes that it will undergo and has developed a strength near its maximum strength.

Ordinarily, lime mortar does not harden

to the final condition of hardness for a great many months and in some cases a number of years, whereas the initial set occurs in about 20 hours when using standard sanded lime mortar, and in our mortar, the time of initial set may be adjusted to take place at any desired time after mixing from five minutes to the time required for standard sand lime mixtures. The term "set" is sometimes used indiscriminately as synonymous with hardness. When so used, it is of course clear, that the final hardness of the material is referred to.

Unless otherwise stated, in the experiments, set forth herein, we have used the standard Gillmore needle in testing for the set of lime mortar. We find that when the large Gillmore needle penetrates to a distance of 2 mm. in the pat the mortar has assumed its set, that is, it is in a condition to receive the second coat. We believe that the Gillmore needle test gives a substantially correct indication of the set; of course, in actual practice, the trowel used in applying the second coat exerts pressure over a very large area whereas the Gillmore needle puts the pressure on a minute spot. In many cases the test pieces are hard and firm when tested with a medium having a large area, such as the hand, although with the Gillmore needle test, the needle will penetrate perhaps a little more than 2 mm. Testing by different methods, as indicated above, there may be some difference in results, but on the whole, the results will be found to approximately correspond. The relation between the penetration of the needle and the suitability of the mortar to receive the second coat has been checked up by practical plasterers.

We have found that quick initial setting properties may be imparted to plastic materials such as hydrated lime and thereby the latter may be successfully used for plastering purposes and for the production of mortars, blocks and the like. We have

found that when hydrated lime or lime putty that has been exposed to the proper proportion of carbon dioxide is mixed with a compound having a sulphate radical to form a plastic mass, the latter acquires quick initial setting properties. Either organic or inorganic sulphate compounds may be used. Among the organic sulphates, aniline sulphate and dimethyl sulphate have given excellent results. However, in the preferred embodiment of our invention, we contemplate the use of the metal sulphates. The proportion of carbon dioxide necessary in the plastic mass for the best results is of paramount importance as will be hereinafter set forth.

In the accompanying figure the curve shows the time of set of mixtures containing carbon dioxide and an inorganic sulphate. The ordinates show the time of set and the abscissæ the amount of carbon dioxide present by weight. This specific curve was plotted from the results obtained by mixing 60 grams of hydrated lime containing varying amounts of carbon dioxide and 1 gram of ferric sulphate and a suitable amount of water. Using different mixtures the curve will, of course, vary somewhat, but in general, the curves will be similar.

Hydrated lime will, on exposure to carbon dioxide, absorb this gas. For the purpose of preparing a quick setting plastic mass in conjunction with the use of an inorganic sulphate, we have found that the percentage of carbon dioxide must be controlled. It is quite easy to introduce too much carbon dioxide and, when this occurs, the hydrated lime loses its capacity to take on an initial quick set when used as an ingredient in a plastic mix, such as a plaster mix. Referring to the accompanying figure, it is seen that when the percentage of carbon dioxide present in the hydrated lime is between 1 and 5½ per cent, the time of set varies through a considerable range from less than one-half hour to less than 11 hours. When the percentage of carbon dioxide is between 1¾ and 3¼ per cent the time of set varies between 4 hours and less than a half an hour. The quicklime from which the results set forth in the curve were derived had the following composition:

|                  | Per cent. |
|------------------|-----------|
| 55 Calcium oxide | 98.00     |
| Iron oxide       | 0.02      |
| Alumina          | 0.30      |
| Magnesia         | 0.45      |
| Silica           | 0.44      |

Using different limes, having different physical and chemical characteristics, the percentages of CO<sub>2</sub> absorbed by the hydrated lime and periods of set, will, of course, be somewhat different and we do not desire to be limited by any definite percentages. The

limitation that we do desire to impose is that the carbonation in conjunction with the use of sulphates, either organic or inorganic, shall produce in the material a quick initial set. The latter is, of course, a relative term but its meaning is entirely clear when taken in connection with the present specification. In general, it may be said that a carbon dioxide content between 1½ and 6 per cent gives satisfactory results and that the best results are obtained with a carbon dioxide-content between 2½ and 4½ per cent. The percentage of carbon dioxide referred to includes the carbon dioxide in the lime from air-carbonation.

The carbonation of the hydrated lime may be carried out as follows: The hydrated lime is placed in a cylindrical vessel provided with baffle plates and containing an opening adapted to receive a tube leading from a source of carbon dioxide. The vessel containing the hydrated lime is rotated by a motor which insures that the hydrated lime flowing over the baffle plates is thoroughly mixed and therefore uniformly treated by carbon dioxide. The carbon dioxide may be introduced with or without the application of external heat. If the gas is introduced into the hydrated lime without the external application of heat, a period of 20 or 40 minutes is required in order to get sufficient absorption of the carbon dioxide to give satisfactory results. The absorption of the carbon dioxide by the hydrated lime usually evolves sufficient heat to accelerate the reaction. In small-scale operations, the radiation of the heat is usually sufficiently rapid to prevent any undesirable overheating and still allow the absorption of the carbon dioxide to occur quickly. However, if the radiation proceeds faster than the generation of heat by the absorption of the carbon dioxide, the absorption may practically cease. In such cases, the heat-content of the hydrated lime may be maintained by external heating to a suitable temperature. In some cases we have found 50° C. satisfactory. The carbon dioxide necessary for the carbonation may be prepared in any desired manner, but at a lime plant the kiln exit gases are conveniently used as a source of carbon dioxide. Limes, which have been exposed to the air until the required quantity of carbon dioxide has been absorbed may be used, in conjunction with a sulphate, to produce a plastic having quick initial setting properties.

The addition of ground calcium carbonate will not produce an initial quick set. We have also found that the carbon dioxide in the carbonate core sometimes present in burned lime is not effective to accelerate the setting of the lime. Our experiments indicate that an over-carbonated hydrated lime cannot be mixed with a fresh-hydrated lime

to produce a quick setting plaster. In our process the quick setting is not a surface change but occurs throughout the mass. A broken block will show approximately the same hardness in the interior as on the surface.

A mortar or plaster which will have a quick initial set may be prepared by mixing carbonated hydrated lime and a sulphate in suitable proportions. Hair, sand, or hair and sand may be added with the sulphate to the carbonated hydrated lime and the entire mass mixed with the required amount of water. What is known as a 1:3 mix, that is, one part of carbonated hydrated lime to three parts of sand may be used but other proportions are suitable and we do not desire to be limited to a mix having any specific composition. It is not necessary that the sulphate be in a very fine state of division or uniformly mixed with the hydrated lime but we have found that the best results are obtained when the sulphate is added in a finely divided condition and is uniformly mixed with the carbonated hydrated lime. Various organic or inorganic sulphates of the type referred to may be used, but we have secured the best results with aniline sulphate and manganese, ferric, and ferrous sulphates. Other sulphates which may be used are those of magnesium, nickel, cobalt, chromium, cadmium, and zinc. These sulphates are typical of those which do not produce an efflorescing compound in reaction with lime. Sodium sulphate is typical of those which produce efflorescence and for this reason is not very desirable.

As a specific example illustrative of our invention the following is given: If hydrated lime containing from 1½ to 6 per cent of carbon dioxide by weight with or without sand or other usual ingredients is treated with an equal weight of water containing one of the above-mentioned sulphates, such as magnesium, manganese or iron sulphate in solution in such amount that the ratio of the dissolved salt to the dry hydrate is one gram to sixty grams, a plaster is obtained which is of normal consistency but which in a few minutes, that is in 5 to 15 minutes after being mixed, takes on an initial stiffening which when subjected to an indentation test by a one-pound Gillmore needle gives a reading of 2 mm. If the ratio of the metallic sulphate to the dry hydrated lime is 1:60 by weight, it is obvious that the resulting plaster sets too quickly, but if the concentration of the metallic sulphate is cut down to 1:120, a plaster is obtained which acquires an initial set in forty minutes or somewhat longer after being mixed. It is therefore obvious that by proper regulation of the quantity of metallic sulphate in the carbonated hydrated lime containing from 1.5% to 6% carbon dioxide by weight, a

plaster may be obtained which will set within any desired time. If the concentration of the metallic sulphate is gradually reduced to zero the time required for set is correspondingly reduced until it approaches the limit set by the hydrated lime containing nothing but carbon dioxide.

The carbonated hydrated lime may be mixed with the finely divided sulphate in a dry state in which case there is no reaction between the mix-constituents until after the water is added. Proceeding as outlined, the sulphate, carbonated hydrated lime, and other ingredients may be mixed at the place of manufacture and thereby a prepared dry plaster mix sent to the trade which requires only the addition of water to be immediately available for use. In a mix prepared as set forth above there is no substantial reaction between the constituents until the water is added. The substances being of such a nature that they are slowly soluble in an alkaline medium, the reaction between the hydrated lime and sulphate progresses slowly, and consequently no setting action is apparent within such a time as to permit the placing of the mortar or plaster in place in the joint or on the surface to be plastered. Ultimately, however, after the plaster is in place, the reaction does progress to such an extent as to produce the setting action.

The following table shows the effect on the time of set of varying amounts of carbon dioxide and sulphate:

| Addition agent               | Per cent addition agent | Per cent $\text{CO}_2$ | Time of set              |      | 100 |
|------------------------------|-------------------------|------------------------|--------------------------|------|-----|
|                              |                         |                        | Hrs.                     | Min. |     |
| $\text{MnSO}_4$              | 1.64                    | 3.56                   | 1                        | 20   | 105 |
| $\text{MnSO}_4$              | 8.20                    | 3.56                   | 2                        | 30   |     |
| $\text{MnSO}_4$              | .25                     | 3.73                   | 3                        | 45   |     |
| $\text{MnSO}_4$              | 5.00                    | 2.00                   | 4                        | 40   |     |
| $\text{MnSO}_4$              | 2                       | 3.5                    | 2                        | 30   |     |
| $\text{Fe}_2(\text{SO}_4)_3$ | 2                       | 3.5                    | 5                        |      |     |
| $\text{Fe}_2(\text{SO}_4)_3$ | 1.64                    | 3.58                   |                          | 9½   |     |
| $\text{Fe}_2(\text{SO}_4)_3$ | 2                       | 3.5                    |                          | 18   |     |
| Aniline sulphate             | 1                       | 3.35                   | set to finger in 10 min. |      |     |
| Hydrated lime alone          |                         |                        | 20                       |      | 110 |
| Prepared gypsum plaster      |                         |                        | 9                        |      |     |

In the above table the percentage of addition agent, and carbon dioxide is figured on the combined weight of the hydrated lime, addition agent, and carbon dioxide. For example, 5% manganese sulphate and 2% carbon dioxide means 5 parts manganese, 2 parts carbon dioxide and 93 parts of hydrated lime.

The test pieces prepared from the above mixtures were molded almost immediately, that is within a minute or two, after water was added to the mix to form the mortar.

Instead of using carbonated hydrated lime as heretofore set forth, putty may also be carbonated by saturating activated carbon with carbon dioxide and distributing the carbon together with a sulphate through the putty mass. It is preferable to use the

carbonated hydrate, but as stated, the putty may also be used.

The mixtures set forth should be applied to the wall within a few minutes after mixing with water. If the mortar is reworked or retempered and it has started to stiffen or set, it will not set again except after many hours. In order to delay the setting action it is usually necessary to add a retarder in sufficient quantities to delay the set and thereby allow the workmen sufficient time to prepare and use the plaster. Suitable retarders are glue, sugar, dextrine, glucose, casein, dried blood, tankage, solutions from tanneries, glycerine, cresol, phenol, pyridin, tannin and the like.

The following table indicates how the use of a retarder, such as sugar, allows the working of the quickest plaster in the manner usually employed by workmen.

In the experiments, from which the results set forth in the following table were obtained, the hydrated lime contained 4.2 per cent of carbon dioxide. Each test piece 25 was made by dissolving the quantity of sugar given in the table and one gram of manganese sulphate in 35 cc. of water. This solution was then added to 30 grams of hydrated carbonated lime and 60 grams of 30 standard sand, after which the whole mass was thoroughly mixed, allowed to stand for 30 minutes, mixed again, and then made into test blocks.

|    | Grams sugar used | Time of set in hours from making of test piece |
|----|------------------|------------------------------------------------|
| 35 |                  |                                                |
| 40 | 0.01             | 7.5                                            |
|    | 0.02             | 7.5                                            |
|    | 0.03             | 3.5                                            |
|    | 0.04             | 3.5                                            |
|    | 0.05             | 3.5                                            |
|    | 0.06             | 3.5                                            |
|    | 0.07             | 3.5                                            |
|    | 0.08             | 3.5                                            |
|    | 0.09             | 3.5                                            |
|    | 0.10             | 3.5                                            |
|    | 0.11             | 5.5                                            |
|    | 0.12             | 5.5                                            |
|    | 0.13             | 5.5                                            |
|    | 0.14             | 5.5                                            |
| 45 |                  |                                                |

50 The time of set, given in the last column, clearly shows the valuable action of the retarder. Without the retarder, the mixes would have stiffened or set inside of 30 minutes. The breaking up of this set by the 55 reworking and forming of the test pieces would have prevented any new set except after several hours. With the quantity of sugar below 0.020 grams, the initial set which had started before the end of thirty 60 minutes was broken up and the new set did not occur until after 7.5 hours. With sugar present in a quantity ranging from 0.03 to 0.1 grams, the initial set did not start during the period of standing and, therefore, a 65 set was obtained in the test blocks in 3.5

hours. With more sugar, 0.12 to 0.14 grams, the final set was delayed to 5.5 hours. Using 60 grams of lime containing 3.35% of carbon dioxide, on the addition of 1% of aniline dissolved in 70 cc. of water and containing 60 milligrams of sugar, the test piece set to the finger in twenty-five minutes.

70 From the above it is clear that the time of set may be increased or decreased by regulating the quantities of carbon dioxide, sulphates, and retarder present. With certain percentages of carbon dioxide and sulphate, no retarder may be necessary. When the percentages are such as to give too quick an initial set, the retarder should be added.

75 The following table shows the importance of the quantity of carbon dioxide in the hydrated lime for the maximum rate of setting. The best pieces were made with 80 60 grams hydrated lime carbonated to varying degrees, 70 grams water, one gram manganese sulphate and 0.08 grams of sugar. No sand was used:

| Per cent carbon dioxide | Time of set in hours |
|-------------------------|----------------------|
| 0.52                    | 20                   |
| 1.88                    | 18                   |
| 2.04                    | 17                   |
| 4.34                    | 2 $\frac{1}{2}$      |
| 4.48                    | 2 $\frac{1}{2}$      |
| 4.72                    | 2 $\frac{1}{2}$      |
| 5.19                    | 9                    |
| 9.91                    | 19                   |
| 10.3                    | 20                   |

90

95

100

105

110

115

120

125

130

100 The term "hydrated lime" as used in the specification and claims includes various kinds of commercial hydrated lime which may vary considerably in its composition. It is intended to include thereunder both calcium and dolomitic hydrated lime. In addition, we intend to cover with this term dry hydrated lime which is a definite article of commerce or lime putty which may be made from dry hydrated lime or from quick lime.

105 In the claims, the term "carbonated hydrated lime" is intended to include any of the above described forms of hydrated lime which have been treated with carbon dioxide, the latter being present either in the combined state or the free state or both.

110 The elements, sodium, potassium, magnesium, aluminum, chromium, manganese, iron, cobalt and nickel appear in series 3 and 4 of the periodic table as devised by Mendeleeff, (see page 2, Van Nostrand's Chemical Annual, 5th ed., 1922). In the claims, by the phrase "a soluble sulphate of a metal in series 3 and 4 of Mendeleeff's periodic table", we intend to cover any soluble sulphate appearing in series 3 and 4.

115 We claim:

1. A plastic material having quick initial setting properties consisting of the reaction products of carbonated hydrated lime and a

- soluble compound having a sulphate radical.
2. A plastic material having quick initial setting properties consisting of the reaction products of carbonated hydrated lime and a soluble inorganic sulphate.
3. A plastic material having quick initial setting properties consisting of the reaction products of carbonated hydrated lime and a soluble sulphate of a metal in series 3 and 4 of Mendeleeff's periodic table.
4. A plastic material having quick initial setting properties comprising the reaction products of carbonated hydrated lime and manganese sulphate.
- 15 5. A plastic material having quick initial setting properties comprising the reaction products of a mixture of a soluble compound having a sulphate radical and hydrated lime containing sufficient carbon dioxide as to aid in imparting to the mixture quick setting properties.
- 20 6. A plastic material having quick initial setting properties comprising the reaction products of a mixture of a soluble inorganic sulphate and hydrated lime containing sufficient carbon dioxide as to aid in imparting to the mixture quick setting properties.
7. A plastic material having quick initial setting properties comprising the reaction products of a mixture of manganese sulphate and hydrated lime containing sufficient carbon dioxide, as to aid in imparting to the mixture quick setting properties.
- 25 8. A plastic material having quick initial setting properties comprising the reaction products of a mixture of a soluble sulphate of a metal in series 3 and 4 of Mendeleeff's periodic table, and hydrated lime containing a sufficient quantity of carbon dioxide, as to aid in imparting to the mixture quick setting properties.
- 30 9. A plastic material having quick initial setting properties comprising the reaction products of a mixture of a soluble sulphate of a metal in series 3 and 4 of Mendeleeff's periodic table, and hydrated lime containing 1½ to 6 per cent of carbon dioxide.
- 35 10. A plastic material having quick initial setting properties comprising the reaction products of a mixture of a soluble sulphate of a metal in series 3 and 4 of Mendeleeff's periodic table, and hydrated lime containing 1½ to 6 per cent carbon dioxide.
- 40 11. A plastic material having quick initial setting properties comprising the reaction products of a mixture of manganese sulphate and hydrated lime containing 1½ to 6 per cent carbon dioxide.
- 45 12. A prepared plaster mix having quick initial setting properties consisting of a mixture of a soluble compound having a sulphate radical and carbonated hydrated lime.
- 50 13. A prepared plaster mix having quick initial setting properties consisting of a mixture of a soluble inorganic sulphate and carbonated hydrated lime.
14. A prepared plaster mix having quick initial setting properties consisting of a mixture of a soluble sulphate of a metal in series 3 and 4 of Mendeleeff's periodic table, and carbonated hydrated lime.
- 70 15. A prepared plaster mix having quick initial setting properties comprising a mixture of manganese sulphate and carbonated hydrated lime.
- 75 16. A prepared plaster mix having quick initial setting properties comprising a mixture of a soluble compound having a sulphate radical and hydrated lime containing sufficient carbon dioxide, as to aid in imparting to the mixture quick setting properties.
- 80 17. A prepared plaster mix having quick initial setting properties comprising a mixture of a soluble inorganic sulphate and hydrated lime containing sufficient carbon dioxide, as to aid in imparting to the mixture quick setting properties.
- 85 18. A prepared plaster mix having quick initial setting properties comprising manganese sulphate and hydrated lime containing sufficient carbon dioxide, as to aid in imparting to the mixture quick setting properties.
- 90 19. A prepared plaster mix having quick initial setting properties comprising a mixture of a soluble compound having a sulphate radical and hydrated lime containing 1½ to 6 per cent carbon dioxide.
- 95 20. A prepared plaster mix having quick initial setting properties comprising a mixture of a soluble inorganic sulphate and hydrated lime containing 1½ to 6 per cent carbon dioxide.
- 100 21. A prepared plaster mix having quick initial setting properties comprising a mixture of manganese sulphate and hydrated lime containing 1½ to 6 per cent carbon dioxide.
- 105 22. The process of producing plastic materials having quick initial setting properties comprising carbonating hydrated lime and treating the reaction-product with a compound having a sulphate radical.
- 110 23. The process of producing plastic materials having quick initial setting properties comprising carbonating hydrated lime until it contains from 1½% to 6% of carbon dioxide and treating the reaction-product with a compound having a sulphate radical.
- 115 24. The process of producing plastic materials having quick initial setting properties comprising carbonating hydrated lime and treating the reaction-product with a soluble inorganic sulphate.
- 120 25. The process of producing plastic materials having quick initial setting properties comprising carbonating hydrated lime until it contains from 1½ to 6 per cent of carbon dioxide and treating the reaction-product with a soluble inorganic sulphate.
- 125 26. The process of producing plastic materials having quick initial setting properties

comprising carbonating hydrated lime and treating the reaction product with a soluble sulphate of a metal in series 3 and 4 of Mendeleeff's periodic table.

and treating the reaction product with a soluble sulphate of a metal in series 3 and 4 <sup>10</sup> of Mendeleeff's periodic table.

- 5 27. The process of producing plastic materials having quick initial setting properties comprising carbonating hydrated lime until it contains from 1½ to 6% of carbon dioxid

In testimony whereof they hereunto affix their signatures.

FRANK C. MATHERS.  
RUSSEL L. HARDY.